

## UNITED STATES PATENT OFFICE.

MILTON L. MOYER, OF SOUDERTON, PENNSYLVANIA, ASSIGNOR, BY DIRECT AND MESNE ASSIGNMENTS, TO MILTON L. MOYER, EDWIN J. PRINDLE, AND BRADLEY STOUGHTON, JOINT TRUSTEES.

## METAL-TREATING COMPOUND AND METHOD OF MAKING SAME.

No Drawing.

Application filed October 9, 1925. Serial No. 61,568.

This invention relates to metal treating and includes a process of treating metals, a compound for use in such treatment and a process of making such compound.

5 The general object of the invention is to produce the compound and the resulting treated metal, and to disclose the method of preparation of the compound, as well as the method by which it is used in treating metal.

10 The present invention is designed particularly to be used in connection with iron, to improve the general qualities of the iron. One of the more particular objects of the invention is to produce a compound found 15 to be particularly useful in increasing the toughness of iron and rendering the iron extremely hard upon suitable tempering.

Another object of the invention is to disclose a method of making the compound 20 and using it in connection with the treatment of iron.

Other objects and features of the invention will more fully appear from the following description and will be particularly 25 pointed out in the claims.

There are many possible embodiments of the invention. For purposes of illustration it is deemed necessary to disclose only one such embodiment which has been found to 30 give excellent results. It is to be understood however, that the preferred embodiment hereinafter disclosed is illustrative only and typical of many possible embodiments.

35 The preferred compound as used at present comprises

soap, eight ounces  
sperm oil, two ounces

40 alum, one-half ounce  
mercury bichloride, one-quarter ounce  
zinc sulfate, one-quarter ounce  
litharge, one-eighth to one-quarter ounce  
carbon, one-eighth to one-quarter ounce.

45 Any suitable form or equivalent of these ingredients may be used. For instance, the soap used is preferably the ordinary yellow soap which is readily obtainable and relatively cheap. In place of the sperm oil its 50 equivalent, spermaceti wax, may be used. Lead sulfate may be used in place of the litharge with fair success, although litharge is preferable. Many forms of carbon, such

as charcoal, or even brown sugar, may be used.

55 In making the compound, the soap is preferably first melted and then the oil or its equivalent in wax is stirred in until a homogeneous mass is obtained. The mixture of the soap and oil or wax provides a fatty substance which may for convenience be termed the base of the compound. After the soap and oil are mixed, the remainder of the ingredients are added. These may be added separately or together, but preferably 60 the dry materials, such as the alum, zinc sulfate, mercury bichloride, and litharge, are first thoroughly pulverized and mixed by themselves, and then added to the fatty substance in small quantities, while the mass is 65 stirred so that all of the ingredients are thoroughly incorporated. If the carbon used is charcoal, or other dry substance, it may be mixed with the litharge and pulverized and incorporated with the other ingredients, 70 but if the carbon be in the form of brown sugar, which at times is somewhat sticky, it is conveniently added to the fatty substance 75

and incorporated with the other ingredients, but if the carbon be in the form of brown sugar, which at times is somewhat sticky, it is conveniently added to the fatty substance before the dry ingredients are added, in order that the sugar may more easily be incorporated. When all the ingredients have 80 been put together and the mass sufficiently agitated so that the ingredients are thoroughly incorporated it is permitted to stand until cool, when it will be found to have 85 a consistency similar to that of soft putty. It will be appreciated that the consistency of the mixture may be controlled somewhat by using a soft soap in conjunction with sperm oil if a soft compound is desired and using a harder soap in conjunction with spermaceti wax if a harder compound is desired.

90 Iron or steel may be treated with the compound in any suitable and convenient manner. As an example of the treatment of small objects, the method of toughening and hardening drill bits and small iron rods may be mentioned. The drills or rods are first heated to a straw color and then immersed 95 in the above described compound. The drills or rods may be left in the compound any desired length of time, but preferably they are left in the compound until thoroughly cool. It has been found that the longer they remain in the compound, the 100 105

greater are the beneficial effects derived from the treatment; that is, if a heated drill is merely plunged into the compound and then withdrawn and allowed to cool in the air, the drill is toughened and upon suitable tempering treatment later will be found to take a good temper, but if the drill is allowed to remain in the compound until thoroughly cool, it is found that the drill 10 has greater toughness and upon suitable tempering later will be extremely hard. Experiments with small bars of iron have developed the fact that if two sections of iron are cut from the same bar and one of them is treated as above described, and then each bar twisted to the breaking point, the untreated bar will break at a distance from the point at which the bar is gripped while the treated bar will stand twice as many 20 turns as the untreated bar and then break at the point where the gripping tool started the shearing of the bar. Drills treated as above described do not break under a twisting force until they have been twisted 25 through a considerable angle.

After the iron articles, such as the above described drills, have been heated to a straw color and then allowed to cool in the compound they may be tempered as desired and it has been found that iron tempered, after being treated, is much harder than the iron obtained from the best methods of tempering now known. Drills tempered after being treated with the compound, by heating to a cherry red and then drawing the temper by water or kerosene have been found to be extremely hard. Drawing the temper with kerosene apparently makes the drills harder than if the 35 temper is drawn with water.

From the foregoing description of the compound, the processes of making and using it and the description of its advantageous effects on iron, it will be seen that 40 applicant has disclosed an invention of large importance which represents a distinct advance in the art. Although a particular and preferred form of making and using the invention has been disclosed, it is desired that these be taken as illustrative merely and that the invention be construed as broadly as the limitations in the claims, taken in conjunction with the prior art may allow.

55 I claim:

1. A metal treating compound including a fatty substance, a bichloride, and a sulfur containing substance.

2. A metal treating compound including

a fatty substance, a bichloride, a sulfate, an oxide, and carbon.

3. A metal treating compound including an emulsifying medium, an oil, a bichloride, and a sulfate.

4. A metal treating compound including an emulsifying medium, an animal oil, a bichloride, and a sulfate.

5. A metal treating compound including a mercury salt and a zinc salt.

6. A metal treating compound including a metal bichloride and a metal sulfate.

7. A metal treating compound including mercury bichloride and zinc sulfate.

8. A metal treating compound including a fatty substance, a mercury salt and a zinc salt.

9. A metal treating compound including a fatty substance, a metal bichloride, and a metal sulfate.

10. A metal treating compound including a fatty substance, mercury bichloride and a zinc sulfate.

11. A metal treating compound including a fatty substance, a mercury salt, a zinc salt, and alum.

12. A metal treating compound including a mercury salt, a zinc salt and alum.

13. A metal treating compound comprising soap, sperm oil, alum, mercury bichloride, zinc sulfate, litharge and carbon.

14. A metal treating compound comprising

soap, eight ounces

sperm oil, two ounces

alum, one-half ounce

mercury bichloride, one-quarter ounce

zinc sulfate, one-quarter ounce

litharge, one-quarter ounce

charcoal.

15. The process of making a metal treating compound which comprises mixing together heated soap and oil and then adding a mercury salt and a zinc salt.

16. The process of making a metal treating compound which comprises mixing together heated soap and oil and then stirring in a metal bichloride and a metal sulfate.

17. The process of making a metal treating compound which comprises mixing soap, adding oil to the mixed soap, while thoroughly mixing the soap and oil, and then stirring in mercury bichloride and zinc sulfate.

In testimony that I claim the foregoing, I have hereunto set my hand this 6th day of October, 1925.

MILTON L. MOYER.